

S. I. CLAWSON.

## PROCESS OF CONCENTRATION OF METALLIFEROUS ORES.

APPLICATION FILED JAN. 2, 1914.

1,240,824.

Patented Sept. 25, 1917.



# UNITED STATES PATENT OFFICE.

SELDEN IRWIN CLAWSON, OF SALT LAKE CITY, UTAH.

## PROCESS OF CONCENTRATION OF METALLIFEROUS ORES.

1,240,824.

Specification of Letters Patent. Patented Sept. 25, 1917.

Application filed January 2, 1914. Serial No. 809,927.

To all whom it may concern:

Be it known that I, SELDEN I. CLAWSON, a citizen of the United States, residing at Salt Lake City, in the county of Salt Lake, 5 State of Utah, have invented certain new and useful Improvements in Processes of Concentration of Metalliferous Ores, of which the following is a description, reference being had to the accompanying drawings and to the figures of reference marked thereon.

My invention relates to improvements in a process of concentration of metalliferous ores by flotation.

15 The object of my invention is to provide a process whereby all of the concentrates can be more readily separated from the gangue by flotation, and in which the oil, gas and other acids used to cause the concentration to rise to the surface of the water are readily saved and used again in the separation of other concentrates.

Another object is to provide a simple, cheap and more effective process for separating the concentrates from the gangue, in which certain acids are used to cause the same to rise to the surface, whereby they may be more readily separated.

In the accompanying drawings—

30 Figure 1 is a side elevation, partly in section, of an apparatus for carrying out my process of separation.

Fig. 2 is a vertical transverse sectional view taken on the line 2—2, Fig. 1.

35 Referring now to the drawings, 1 represents a hopper which is supported in any desired manner and has its lower end in communication with a horizontally arranged elongated mixing chamber 2, in which is mounted a horizontally arranged rotatable shaft 3, carrying the agitating blades or teeth 4, for agitating the ore as it leaves the hopper, as will be hereinafter more fully described.

45 The hopper 1, as shown, is connected to one end of the mixing chamber and connected to and in communication with the opposite end of the chamber is a pump casing 5, in which is mounted the centrifugal

50 pump 6 on the shaft 3. The said shaft extends entirely through the pump casing and is provided with a pulley 7, by means of which the pump and the agitator are rotated, as will be readily understood.

55 The pump casing has its lower end connected to the injector 11, which leads into

the horizontally arranged pipe 9. The said pipe, beyond the injector 11, is provided with a contracted passage 11', and beyond the contracted passage the pipe 9 is made in 60 a zigzag form to cause a greater agitation of the ore, as is indicated by the reference numeral 12. The zigzag passage is connected to and in communication with the chamber 14, which has its upper end above 65 a line with the entrance of the zigzag passage and of a transparent material, whereby the action within the chamber can be readily seen. The chamber 14 has, in communication with the opposite end, the concentrating 70 box 15 and said communication being in a line with the upper end of the zigzag passage, as clearly shown in dotted lines, indicating the water line in the chamber.

The lower end of the chamber 14 is provided with a cock 16, by means of which the rock and other earth deposits can be readily drawn off. The lower end of the concentrating box 15 is provided with a cock 17, whereby the concentrates can be readily 80 drawn therefrom. The top of the chamber 14 is provided with a downwardly disposed portion 14', which is directly above the junction of the chamber 14 and the concentrating box 15.

85 The pipe 9, just above the injector 11, has a pipe 18 in communication therewith which has connected thereto a horizontally arranged pipe 19 leading to the gas generator 20, whereby the gas is sucked from the 90 pipe 18 by the injector 11. Connected to the pipe 19 is a pipe 21, which has its upper end in communication with the upper end of the concentrates box, whereby the unused gas is conveyed to the pipe 19 and used again. 95

Above the hopper 1 is an ore hopper 21', which is adapted to discharge into the said hopper 1. Above the hopper 1 is an oil tank 22 and the acid supply tank 22', which discharge into the hopper 1, as will be herein- 100 after more fully described. The salt water tank 23 is placed above the hopper 1, and is adapted to supply water thereto, as the ore, oil and acid is fed thereto, as will be herein- 105 after more fully described.

In operation, the ore, water, oil and acid are fed to the hopper 1, as heretofore described, and pass into the mixing chamber 2, where they are thoroughly mixed by the agitator blades or teeth 4, and the mixture 110 is then carried to the centrifugal pump where it is more thoroughly mixed. The

mixture is forced from the centrifugal pump through the injector to the horizontal tube. As the mixture passes from the injector gas is drawn inwardly through the 5 pipe 18 and mixes therewith. The mixture of ore, water, gas, oil and acid is then driven through the restricted passage under pressure, where it is more thoroughly mixed. It next passes through the zigzag passage and 10 enters the separating chamber 14. The concentrates rise to the surface of the liquid in the chamber by the aid of the buoyant materials added to the charge and the concentrates flow over the lip into the concentrates 15 box 15. The rising and separating of the concentrates are further assisted by the air or gas passing in the same direction under the partition 14'. The rock or earthy ingredients unaffected by the buoyant materials sink to the bottom of the chamber 14 20 and are drawn off from the cock.

When gas is used in the operation, the gas is generated in the generator 20, as heretofore described, but when air is to be used, 25 in place of gas, the generator 20 is closed and the pipe connections are opened by the valves 24 and 25 to the atmosphere. If the ore requires calcites, it is fed into the ore hopper 21' from the tank 26, above the 30 same. Heat is applied in the form of steam, which also adds buoyancy to the concentrates.

In my improved process, the ore is first 35 thoroughly mixed with a saline solution, oil and an acid and is then thoroughly aerated or charged with gas, all of which will increase the buoyancy of the concentrates and when they enter the chamber 14, they float upon the surface of the solution, 40 and upon gas pressure, which is present above the solution, a still greater buoyancy is given to the concentrates. The gangue sinks to the bottom of the chamber 14, while the concentrates float over the portion be-

tween the chamber 14 and the concentrates 45 box 15, where the concentrates are removed, as heretofore described. The solution in the chamber 14 is heated by steam which gives still greater buoyancy to the concentrates. Any machine consisting of an in- 50 closure for maintaining a gas above the surface of the liquid in the flotation tank would answer the requirements of my new process.

Having thus described my invention, what 55 I claim is:

1. The herein described improvement in concentrating ores by the flotation process which consists in mixing the pulverized ores with a saline solution and oil, charging the 60 mixture with gas, by throttled injection discharging the pulp thus formed into a closed separating chamber or tank, the supply of gas being sufficient to create a body of gas under pressure in the upper portion of said 65 tank and returning the gas from the region of froth formation to the region of pulp and gas injection.

2. The herein described improvement in concentrating ores by the flotation process 70 which consists in mixing the pulverized ores with a saline solution, adding gas and oil under injection, forcing the mixture of pulp into one side of a closed separating chamber under pressure, collecting the concentrates from the opposite side of said chamber for withdrawal, leading the surplus gas under pressure from the side of the separating chamber opposite its point of entry back to the point of injection for reuse in 75 80 connection with a new supply of mixed ores.

In testimony whereof, I affix my signature in the presence of two witnesses.

SELDEN IRWIN CLAWSON.

Witnesses:

JOHN H. BURROWS,  
LESTER MERRILL.